

[54] HIGH SHEEN BIFILAMENT YARN AND  
ELASTIC TEXTILE ARTICLE THEREFROM

[76] Inventors: **Ralph W. Schuettler**, 12800 Percival St., Chester; **Garland L. Turner**, Rt. 1, Box 158-A, Chesterfield; **George H. Collingwood**, 3202 Clay St., Hopewell, all of Va.

[22] Filed: **Feb. 18, 1971**

[21] Appl. No.: **116,631**

## Related U.S. Application Data

[62] Division of Ser. No. 733,557, May 31, 1968, abandoned.

[52] U.S. Cl. .... **57/140 J**, 161/177, 264/177

[51] Int. Cl. .... **D02g 3/22**

[58] Field of Search ..... 57/140 J; 264/167, 264/174, 177; 161/177

## [56] References Cited

## UNITED STATES PATENTS

3,308,221 3/1967 Opfell ..... 264/174

Primary Examiner—John Petrakes  
Attorney—Luther A. Marsh

## [57] ABSTRACT

A bifilament yarn comprising two symmetrical lobes fused so that the concave sides intercept at angle  $\theta$  ranging from  $41^\circ$  to  $54^\circ$ . The yarn has a broad concave area and a narrow edge area of convex shape and preferably a modification ratio of between 1.65 and 2.05. This bifilament yarn, textured and non-textured, semi-dull and bright, when converted to plain knit hosiery has a luster in the range of 6.6 to 21 (K/S  $\times$  100) units. The textured and non-textured plain knit textile articles consisting of the bifilament yarns of this invention after repetitive elongations of 25 percent have 150–300 percent greater work of recovery and equal improvement in resistance to sagging and wrinkling than other cross-sectional configurations. The bifilament yarns are prepared by melt spinning thermoplastic homopolymers having a relative formic acid viscosity of 25 to 60 at a temperature of 250°–280°C through twin orifices separated from each other for a distance of 0.05 to 3.0 mils.

7 Claims, 20 Drawing Figures



PATENTED SEP 25 1973

3,760,579

SHEET 1 OF 4



FIG. 1



FIG. 1A



FIG. 2



FIG. 3

PATENTED SEP 25 1973

3,760,579

SHEET 2 OF 4

**FIG.4**



**FIG.5**



**FIG.6**



**FIG.7**



PATENTED SEP 25 1973

3,760,579

SHEET 3 OF 4

**FIG.8**



**FIG.9**



**FIG.10**



**FIG.11**



**FIG.12**



**FIG.13**





FIG. 14



FIG. 15



FIG. 16



FIG. 17



FIG. 18



FIG. 19

F.T. = FALSE TWIST

## HIGH SHEEN BIFILAMENT YARN AND ELASTIC TEXTILE ARTICLE THEREFROM

This is a division of application Ser. No. 733,557, filed May 31, 1968, now abandoned.

### BACKGROUND OF THE INVENTION

Ladies' stretch hosiery have usually been made from false-twisted round cross section yarn or bicomponent yarn where one component is a homopolymer and the other component is a copolymer arranged either side by side with the homopolymer or as a core in a sheath and core arrangement. Such yarns, while finding utility in ladies' hosiery, have a disadvantage in that three or more sizes are required to cover the range of sizes 8-½ to 11-½. This range of sizes amounts to about 99 percent of the ladies' hosiery consumption in the United States. Additionally, various cross-sectional types such as trifilament, triangular, Y-cross section, star cross section, polygonal, and the like, have been employed to achieve decorative effects in these hosiery. When these conventional yarns are employed, three or more sizes are required to cover the practical range of hosiery sizes, and generally, the modified hosiery has either too dull an appearance or too much glitter with the latter having utility only for its novelty effect.

There has long been a need for a true stretch hosiery where one size will fill the majority of end-use requirements and which has sufficient luster and sheen to be desirable for formal wear without being too garish for everyday and business use. It is also highly desirable to produce a true stretch yarn having adequate power of recovery to maintain a good fit without wrinkling or becoming permanently deformed under severe bending action, such as deep-knee bends. Additionally, hosiery yarns made from two components, a homopolymer and a copolymer, are expensive and difficult to produce. Thus, there has long been a need to produce a stretch yarn which avoids the described problems, and more particularly, it has been desirable to produce said yarn from a single homopolymer.

In an attempt to simulate some of the geometric forms of natural fibers, various configurations including bifilament yarns were produced almost four decades ago from man-made cellulosic fibers as disclosed in Swiss Pat. No. 145,408 dated Feb. 28, 1931. Since this time, several patents have issued showing various configurations representing a range of fiber types which have two or more lobes. For example, U.S. Pat. Nos. 3,156,607 and 3,131,427 illustrate yarn configuration which are essentially bilobal. Thus, the prior art is replete with patents showing various types of bilobal yarns yet none of the patentees recognized the critical nature of the angle of intercept between the two lobes which is essential in producing a high sheen hosiery yarn that does not have a garishness related to excessive sparkle.

Additionally, when such multilobed forms are used in ladies' hosiery irrespective of the texturing method employed, three or more sizes of stretch hosiery are required to cover the range of consumer sizes. Indeed, to have truly satisfactory fits in stretch hosiery, five sizes are judged by independent laboratories as being necessary to suit most consumer requirements for a comfortable as being necessary to suit most consumer requirement for a comfortable and attractive fit.

There has been still another problem with prior art yarns in that the stretch qualities on repeated stretching

of hosiery results in continued loss of the original stress-strain properties and sagging or wrinkling of the hosiery may occur, particularly at the ankle section and knee section. With the foregoing discussion in mind, the provision for a homopolymer yarn which possesses the desired appearance factors as well as the desired stretch properties represents a substantial improvement in the art.

### SUMMARY OF THE INVENTION

The product of this invention involves a thermoplastic homopolymer fused into an oblong shape having two symmetrical lobes fused so that the concave sides intercept at an angle  $\theta$  ranging from 41° to 54°, preferably 42°-52°. The bifilament yarn has a broad concave area and a narrow edge (convex) area so that when said yarn is placed in a knit structure, the broad concave areas become aligned facing each other at stitch crossing points to present a convex or edge area to view and twist 90° or more to present the concave or broad areas to view in the loop sections. Light reflects from each concave area presented to view in the loop areas as a minute point flash and the alignment of these minute point flashes result in a sheen or opalescence which is enhanced in bright yarns and reduced if a delusterant is present. Because of its geometrical configuration false-twist bifilament yarn has twice the number of twists trapped in each loop and twice the number of point flashes; therefore, an enhanced luster or sheen is obtained in plain-knit hosiery.

Likewise, this twist trapped in each loop of the knitted structure gives greatly increased multidirectional elastic properties to the grid structure since each twist in each loop, coarse and wale becomes a multiple of the total number of loops of the grid structure thereby greatly enhancing its elasticity.

The preferred modification ratio is 1.65 to 2.05 and more preferably 1.75 to 1.95 and the tip radius is generally 0.9 or greater. The bifilament yarns, textured and non-textured, semidull and bright, when converted to plain knit hosiery as an undyed boardered structure have luster values as follows:

|                     |                            |
|---------------------|----------------------------|
| Bright Non-Textured | 9 to 16 (K/S × 100) units  |
| Bright False-Twist  | 12 to 21 (K/S × 100) units |

These high luster values are due to alignment of minute point flashes resulting in a high glossy sheen termed the "glace look" or "wet look" for bright yarns. This high sheen and uniform luster has not thus far been obtained in prior art knitted structures.

The preferred process for producing the yarn as above described involves employing a polyamide having a relative formic acid viscosity of between 25 and 65 which is extruded through a pair of spinnerette orifices having a distance between said orifices of 0.5 to 3.0 mils, preferably 1.0 to 2.5 mils. Nylon 6 is spun at a temperature of between 250° and 280°C, preferably 265° to 275°C, and nylon 6,6 is spun at approximately 10° higher temperature. The polyamide relative formic acid and the distance between the spinnerette orifices are the two major variables as indicated hereinafter in Table 1. With an increase in relative formic acid viscosity, the modification ratio increases and the angle of intercept decreases and the luster values increase. Thus, a sparkle look is produced and the desired high sheen "glace look" is lost. It is noted, also, that the temperature of the polymer melt must be considered. As tem-

perature increases, the modification ratio decreases. Additionally, at too high a temperature, drips, breaks and wraps may appear, which are undesirable in the processing of such fibers.

Thermoplastics in general can be employed for producing bifilament yarns, but because of their excellent dyeing properties and good optical properties, polyamides usually are preferred for the production of bifilaments in accordance with this invention. Preferred polyamides are poly-e-caprolactam (nylon 6), polyhexamethylene adipamide (nylon 6,6), and the polyamides made by condensation of p,p'-bis(para-aminocyclohexyl)methane with dodecanedioic acid to produce the polyamide poly[bis(p-aminocyclohexyl)methane dodecamide].

The bifilament yarns disclosed as the invention herein have utility in transport upholstery and apparel end uses because of the high elasticity of the knitted structure and the high glossy sheen or "glace look" which characterizes knitted textile articles made from bright bifilaments.

#### BRIEF DESCRIPTION OF THE DRAWINGS

FIG. 1 is a cross section of the spinnerette orifices employed to extrude the bifilament yarns of the present invention.

FIG. 1A is a cross-sectional view representing the bifilament yarn of this invention illustrating how the angle of intercept  $\theta$  is measured.

FIG. 2 illustrates graphically the relationship between the optical properties of the filaments as a function of the angle of the bifilament intercept point versus the modification ratio.

FIG. 3 is a graph illustrating the luster of bifilament yarns of this invention plotted against the modification ratio. These data illustrate the change in sheen between false-twist and normal yarn. The dotted lines show the range of modification ratio which produces the preferred high sheen yarn.

FIG. 4 is a photograph illustrating, at 320 magnifications, representative cross sections of undrawn bifilament yarns of the present invention which have a modification ratio of 1.7.

FIG. 5 is another photograph at 320 magnifications of other bifilament undrawn cross sections which have a high sheen "glace look" when the yarn is placed in a sheer fabric. Generally, above this modification ratio of 2.0, a transition to the sparkle look occurs.

FIG. 6 is a photograph at 560 magnification of a typical cross section of drawn bifilament yarns having a modification ratio of 2.3 to 2.4.

FIG. 7 is a photograph at 900 magnifications of a drawn bifilament yarn having a modification ratio of 2.8 to 2.9.

The yarns of FIGS. 6 and 7 are outside the critical range required to obtain a "glace look".

FIG. 8 is a photograph illustrating the unique property obtained by combination of bifilament geometry with a false-twist operation. This illustrates the alignment of the concave surfaces at stitch cross-over points and the twist which in the loop part exposes the broad parts of the concave surface to view. This additionally illustrates the aligned rows of point light reflections from concave surfaces to give the unique sheen which can be observed. The magnification of FIGS. 8 through 13 is 36X.

FIG. 9 is a bifilament yarn in jersey knit hosiery which was not false-twisted. There is similar twist entrapment and alignment of the light reflective areas as in FIG. 8.

FIG. 10 is a photograph of a round cross-sectional yarn which is false-twisted and knit into hosiery. It can be observed that the light reflective areas are completely random, there is no twist between the stitches, and the yarn tends to curl back on itself rather than be twisted between the stitches.

FIG. 11 is a photograph of round monofilaments of plain knit hosiery. It also lacks the properties of twist entrapment and luster effects characteristic of bifilament yarns as illustrated in FIG. 9.

FIG. 12 is a photograph of stretch hosiery of round cross section, bi-component filaments. Again, there is no alignment of the light areas in the yarn. Consequently, there is no luster or sheen, or enhancement of the elasticity from twist trapped between stitches.

FIG. 13 is a photograph of mesh hosiery tuck stitch made from trilobal or triangular shaped yarns. As can be observed, the light reflection areas are random and significantly larger than those illustrated in FIGS. 8 and 9. Such yarns while suitable for many novelty end-uses have utility only as novelty yarns because of the garishness of the luster.

FIG. 14 is a graph illustrating the force required to elongate a bi-component stretch yarn after one cycle of elongation, and, after six cycles of elongation. The stretch direction was lengthwise and the test sample was ladies' hosiery with plain knit construction.

FIGS. 15 and 16 represent the same test parameters as for FIG. 14 except that FIG. 15 represents false-twist bifilament yarns of this invention which have superior elastic properties over that for FIG. 14 and FIG. 16. FIG. 16 represents false-twist round cross section nylon 6 yarn.

FIGS. 17, 18 and 19 represent, respectively, leg sections of ladies' hosiery made from false-twist bifilament yarn, false-twist round filament yarns and round cross section bicomponent sheath and core yarn. The nature of the test data illustrated in these figures is similar to that described for FIGS. 14, 15 and 16, except the measurement is in the transverse direction.

#### DESCRIPTION OF THE PREFERRED EMBODIMENTS

The bifilament yarns of the present invention preferably are spun from a polyamide such as nylon 6 or nylon 6,6 directly from a continuous polymerization system wherein the polymers are melted prior to extrusion using an extruder or a melter. The molten polymer is then extruded through a pair of orifices in close proximity to each other as depicted in FIG. 1 by capillaries 1 and 3. These capillaries are separated by the portion 2 which is preferably an integrate portion of the spinnerette plate 6. The molten polyamide polymer enters through an entry orifice denoted at 5 and is divided into separate streams on contacting metallic portion 2. The distance between orifices 1 and 3 should be between 0.5 to 3.0 mils. The distance when less than 0.5 mils results in the separator portion 2, too weak to withstand the extrusion pressure. Should the distance between orifices 1 and 3 exceed 3.0 mils, one then enters the region of a sparkle effect and the preferred "glace look" is not obtained. The length of spinnerette orifice 4 should generally be in the region of 0.8 to 4 times the

diameter of the spinnerette orifices 1 to 3, preferably a length to diameter ratio of about 1.2 should be employed.

The yarn product of the present invention has a "glace look" which has been described as a "wet look" when fashioned into articles such as ladies' hosiery and other sheer garments. This appearance is achieved only when critical parameters are observed during the production of the bifilament yarns of this invention. It is essential that the yarns intercept at an angle of between 41° and 54° of the joined filaments. It is also preferred that the yarns have a modification ratio ranging from 1.65 to 2.05. At an intercept angle of greater than 54°, too low a luster is obtained and twist is not trapped between the filament loops to achieve the desirable elasticity properties in knit structures. At an angle of intercept below 41°, the yarn exhibits a sparkle effect and does not have the glace look and desirable opalescent sheen of the product made in accordance with this invention.

The angle of intercept is determined by completing the two circles outlined by the filament lobes 12 and 14, then completing a line bisecting the center of the circles and the point where the circles intercept as shown in FIG. 1A. The angle of intercept is the angle  $\theta$  between the horizontal line passing through the center and the line drawn to the intercept point.

The modification ratio is determined by dividing the minimum width at the point of upper and lower intercept points of the two circles into the length or the distance to the outer perimeter of the two circles. The relationship between the angle and the modification ratio is given in FIG. 2 wherein it is illustrated that as the modification ratio decreases, the higher the angle of intercept.

As can be observed in FIG. 2, the glace appearance coincides at an angle of intercept between approximately 38° and 56°, the area represented by ABCD. At a lower angle of intercept, the glace look is lost and a sparkle effect occurs. At a broader angle of intercept than 54°, there is insufficient luster and the bifilaments lose most of their ability to align face to face at stitch cross-over points, the condition which imparts twist to said bifilaments in the loops between stitches. Therefore, they lose their luster, but most important, they lose their elasticity because of inability to trap twist between each stitch in the knitted structure. It is especially desirable that an angle of intercept be present on both sides of the bifilament yarns so that the twist is always trapped between stitches regardless of which side of the concave surfaces align at the stitch crossing points.

In FIG. 3 is shown a plot of the modification ratio versus luster. Luster is ascertained by measuring light reflectivity with a "Color Eye" manufactured by the Instrument Development Laboratories, Attleboro, Massachusetts. The reflectivity is expressed by the Kubelka Munk equation where:

$$(K/S) = ([1 - R]^2/2R)$$
 where  $R$  = reflectivity ascertained with the "Color Eye" at 557 millimicrons. The method for ascertaining the reflectance has been described in "Color and Business, Science and Industry" by D. B. Judd; John Wiley and Sons, New York, New York, 3rd printing, February 1967, pp. 434-438. As can be observed in FIG. 3, the luster values of significance are from 9 to 21 ( $K/S \times 100$ ) units, preferably 10 to 18 ( $K/S \times 100$ ) units. For false-twist bifilament yarns, the luster values are quite significantly higher than non-textured bifilament yarn made into hosiery. This is due to the presence of approximately twice as many concave reflection points in each stitch loop of textured over the non-textured bifilament yarn. Hosiery fashioned from the textured bifilament yarn have luster values of 14 to 21 ( $K/S \times 100$ ) units. The presence of this additional reflective surface or additional number of reflection points results in a considerable enhancement of the desirable "glace look" over that obtained from the same hosiery made from non-textured bifilament yarns. This enhancement of the glace look by a panel jury evaluation of skilled colourists amounts to 200 to 300 percent increase in the apparent sheen or luster values observed. Non-textured bifilament yarn has a luster value of 8 to 16 ( $K/S \times 100$ ) units. At lower values than the indicated range of bright luster, insufficient luster is present to produce a sheen effect. At higher luster values, as, for example, greater than 16 for the non-textured and greater than 21 for the false-twist hosiery, there is excessive sparkle in the hosiery which tends to limit their utility to novelty end uses.

Generally, within the scope of the luster values indicated, and as shown in FIG. 3, this hosiery is quite acceptable to be worn in everyday office use and still quite attractive and desirable for formal wear. The luster values for semi-dull yarns having the same modification ratio as bright yarns are quite different and only a low level of surface reflectivity is obtained. The major effect is a significant increase in cover due to the visual appearance of the broad concave surface in the loop section of the knitted structure. The increase in cover is 10-20 percent greater than round cross section yarn of the same denier.

A better appreciation for the critical influence that the angle of intercept and modification ratio of the yarn has upon appearance and the performance of the yarn of this product of this invention can be recognized from an investigation of FIG. 4 through FIG. 19. FIGS. 4 to 7 are photomicrographs of cross sections of bifilaments illustrating products of the invention compared with bifilament cross sections that are outside of the invention. The modification ratio of the cross sections shown in FIG. 4 is 1.7 and as can be observed there is only a slight distinct concave surface. Thus, the bifilaments having values below 1.5 and are not concave and generally have neither luster nor the elasticity desired. FIG. 5 is a cross section having a modification ratio of 2.0 which represents the upper limit beyond which excessive sparkle occurs. FIGS. 6 and 7 have modification ratios substantially greater than 2.0 and thereby representing yarns outside the scope of this invention.

FIGS. 4 and 5 illustrate the cross section of undrawn yarns and FIGS. 6 and 7 illustrate a cross section of drawn yarn. As can be observed, undrawn and drawn

cross sections at equivalent magnification have identical geometric cross sections.

Again, when referring to FIG. 1A and FIGS. 4 through 7, it can be noted that when the circles are completed, as indicated in FIG. 1A for circles 12 and 14, the total area of this circle is determined and their measured perimeter is divided into the perfect circle enclosing the measured area. From this arrangement their degree of circularity can be ascertained. Preferably the yarns of this invention have a degree of circularity of greater than 0.9. Bifilaments having a substantially larger deviation from circularity do not have the same sheen and knitting is difficult because of the tendency of such yarns to break out from back-up of twist at the needles.

The performance of hosiery fashioned from bifilament yarns made in accordance with this invention is compared with hosiery made from other yarns in FIGS. 8 through 19. These comparisons are made on the knitted structures since the unusual properties of light reflectivity and elasticity can be observed, and measured only after the yarn is placed in a fabric construction. It should be emphasized that hosiery are used as a common example; however, bifilament yarns react in a similar manner in other jersey knit structures as well as, tricot knit structures, mesh or tuck stitch structures, and rib stitch structures.

FIG. 8 illustrates a section of hosiery fashioned from bifilament yarns having a modification ratio of 1.8. The yarn has 31 turns per inch of twist imparted thereto, utilizing a Leesona 553 Superloft machine. It is knitted into the hosiery using S and Z twist in alternate courses. It can be observed from FIG. 8 the light areas are short in length due to the twist of bifilament yarns between stitches; however, as can be noted, the light areas are all on an approximate similar plane. This results in a diaphanous, luminous sheen, which has been characterized as the "glace look." As the modification ratio of bifilament yarns is increased, the length of the light flashes increases. As the intensity of the light at these points increases, each individual light-colored point results in a scintillation point, and the luminous sheen effect is replaced by a sparkle effect. Between each stitch it can be noted that the bifilament yarns twist 90 degrees first to present a flat plane to view and over the course of the twist, at least another 90 degrees for a total of at least 180 degrees to present two concave planes to view. It is this twist superimposed upon the false-twist stretch that lends sufficient elasticity to the hosiery so one size will span the range of sizes for most consumer end uses.

Additionally, as the stitches in FIG. 8 are stretched, the twist that is trapped between the stitches in the manner stated above gradually untwist and when tension is released, these twists rewind. After stretching, particularly in areas of hosiery where elongations ensue, that is, the areas which have greater propensity to sag or wrinkle, the twist which has been unwound as the individual stitches are stretched out, rewind into a normal configuration and provides additional force superimposed on that from the false-twist crimp. Thus, the combined forces, at low elongation, are adequate to hold the hosiery firm to the ankle or firm to the knee without any evidence of sagging or wrinkling. Moreover, such hosiery resists elongation on repetitive cycling.

In FIG. 9, a bifilament yarn the same as in FIG. 8, except without false-twist, illustrates that all light reflection areas are located at relatively precise points in the center of the plain-knit stitch and along the sides of the stitch. Thus, the bifils present the intercept point on a flat plane in the direction of the light and in the direction of the observer's view. In a comparison between the false-twisted and non-false-twisted yarns, it can be observed that the light areas and stitches are more uniform for the non-twisted yarn, and that the light areas are in a precisely aligned plane. It is this alignment of the reflection areas, which results in the smooth luminous sheen. This may be compared with round cross section yarn in FIG. 11 which exerts no twist entrapment and has essentially no light reflective areas. Additionally, it may be compared with a trifilament yarn cross section in a mesh knit as illustrated in FIG. 13, where the point flashes extend over the long length of the tuck stitches and over broad areas of the standard jersey knit stitches. These broad areas of light reflection promote too much sparkle for most end uses, particularly for office wear and additionally as can be noted, there is less or no twist entrapment between stitches in FIG. 13.

FIG. 12 illustrates a time exposure for round cross section bicomponent elastic yarns. As can be observed, only small sparkle areas are obtained, and if it were not for the lengthy time of exposure, this sparkle could not be observed. Additionally, as can be observed, there is no twist entrapment between the stitches.

In FIG. 13 it can be observed that there is a bright sparkle in the center stitch. It is these large point sparkles that follows the entire length of the stitch which would seen to indicate there is relatively low level of change in planes of the reflecting surface. Therefore, no significant improvement in elastic properties or sheen could be expected from the yarn as illustrated in FIG. 13. Additionally, the sparkle is too bright except for formal occasions.

FIG. 14 illustrates the stress-strain characteristics of a plain knit hose manufactured from a commercial bicomponent round fiber after one cycle and after six cycles. As can be observed, there is almost complete loss of stretch power after six cycles, particularly at 3 percent elongation. Moreover, the values at 5 percent elongation are quite low. However, after these initial elongations there is a rapid increase in the gram loading for small increases in the elongation. It is this rapid increase which is undesirable because there is too much of a load for a given degree of stretch. This type of loading causes an uncomfortable effect on the part of the wearer as well as impart stresses to the individual filaments so that a sudden pick on impact will probably result in a run in the hosiery or garment.

FIG. 15 illustrates the lengthwise extension versus stress-strain load for a hose constructed the same as in FIG. 14 except the bifilament yarn of this invention which has been false-twisted was employed. As can be noted, the hose has a definite initial loading that is still higher after six cycles of extension which slopes upward at a substantially lower rate than that described in FIG. 14. Thus, it has a relatively uniform stretch characteristic maintaining a definite power after repetitive stretching sufficient to avoid wrinkling or sagging of the hosiery.

FIG. 16 represents hosiery processes in identical manner to that illustrated in FIG. 15 with the only dif-

ference being round cross section versus bifilament yarns. Again at 3 percent elongation, after six cycles, there is no power left in the yarn and sagging or wrinkling can occur. Additionally, there is considerable greater drop in the load at 5 percent elongation from the first to the sixth cycle. Generally there is a slower increase in loading with a substantial increase in elongation for the round false-twist yarn than that for the bifilament yarn, as illustrated in FIG. 15, when tested in a lengthwise direction.

False-twist triangular or trilobal cross section yarn is converted into hosiery and processed in identical manner to that as illustrated in FIG. 15 with the only difference being round cross section bifilament yarn versus the round cross section of FIG. 16. Again this cross section exhibits very low load capacities after six cycles which is similar to that for round cross section false-twist yarn, except that at 10 percent elongation and above, loading is very rapid, even more rapid than that illustrated in FIG. 15. This would cause an uncomfortable effect on the part of the wearer as well as stress individual filaments to increase the potential of runs or breakage of the filament from sudden picks or impact.

FIG. 17 illustrates a bifilament yarn in the transverse direction. Comparing FIG. 17 with FIG. 15, it can be observed generally there is a far lower increase in loading in the transverse direction for a given degree of elongation than there is in the lengthwise direction. It is, however, an unexpected advantage of the bifilament yarn, that it has a definite and significant loading capacity even at elongations as low as 3 percent which still remain adequate after six cycles of extension.

FIG. 18 shows exactly the same transverse stress-strain curve for a false-twisted round cross section yarn. As can be noted at low elongation, 3 to 5 percent after six cycles, the false-twist yarn has essentially no load-bearing capacity. Therefore, it would tend to wrinkle. In a similar manner, a triangular cross section false-twisted yarn shows essentially the same initial transverse stress-strain curve as that for round cross section, and then very rapidly loads which is an indication of limited and narrow elastic characteristics.

FIG. 19 illustrates a bicomponent yarn in a transverse extension. This yarn also has very low-bearing capacities throughout the range tested up to 25 percent elongation. Again, if wrinkling should occur, it more probably would occur with the bicomponent yarn of FIG. 19 than with the yarn of FIG. 18, and especially with yarn of this invention illustrated in FIG. 17.

From the foregoing illustrations and comparisons made in connection with the drawings, it can be seen that, in general, the luster of bifilament yarns is a function of the modification ratio whether a "glace look" or a sparkle effect is obtained. Other configurations show quite different luster effects and do not normally demonstrate the silky high sheen characteristic of the modification ratio of between 1.65 and 2.0, which is illustrated in FIGS. 2 and 3. Many end-uses of knit apparel structures require a low degree of transparency. To achieve this effect, anatase titanium dioxide is dispersed in the monomer or at some point prior to completion of the polymerization cycle in the amount of 0.3 percent of  $TiO_2$  by weight of polymer for semidull articles and 2.0 percent by weight of  $TiO_2$  by weight of polymer for full-dull articles. This delustering quality is desirable for its hiding power, but frequently it has undesirable chalkiness or grayishness which decreases the

aesthetic properties of the textile article containing said delusterant. Thus, when the bifilament yarn of this invention is made into knit textile articles, an enhanced warmth of appearance and aesthetic properties is obtained. The delustered yarn has 10-20 percent greater cover on a standard hosiery form as compared with round cross sections of equivalent denier. The high luster obtained for bright yarn has the further advantage in that the high degree of reflectivity which is obtained significantly reduces the apparent soiling as compared with round cross sections and triangular cross sections.

The following examples further illustrate the invention.

#### EXAMPLES 1 - 14

The bifilamentary yarns of the present invention were prepared from polycaproamide pellets of 50 to 55 relative formic acid viscosity which were spun at a temperature of 255° to 260°C from a melter through twin spinnerette orifices, 10 mils in diameter by 10 mils in length and separated from each other at a minimum distance of 2 mils. The spinnerette employed had a counterbore angle of 60° as indicated by reference numeral 5 in FIG. 1. The molten polymer entered the spinnerette counterbore at the rate of 4.78 grams/minute/bifil filament. There were four spinnerettes per stack, each spinnerette producing two strands of bifilament yarn and each spinnerette was separately metered. Thus, eight strands of bifilament yarn were produced per quench stack. The yarn was quenched 3 inches below the spinnerette face with quench air entering at the temperature of 41°C and traveled uniformly transverse to the filaments, at the rate of 10 linear feet/min. for a distance of 95 inches from the point of initial gas contact with the filaments. The yarn then entered a round quench stack of about 7 inches in diameter, thence over a lubrication roll where finish was applied at about 8 to 10 percent by weight of yarn. The yarn was then taken up on a winder having two cops per sleeve and using four sleeves per winder making a total number of eight ends per winder having 4.7 pounds/cop or 9.4 pounds/sleeve. The speed of take-up was 1,950 feet/min. for the undrawn yarn. The bifilament yarn was then placed on drawtwisters passed 1.5 wraps around an Armstrong Rubber Compound 732 cot roll, thence 4 wraps around a draw roll, thence to a cylindrical core where a filling wind or pineapple wind was employed for hosiery. A warp wind was employed for tricot and other sheer-type fabric. The rubber cot roll employed had a shore hardness of 50. A higher value resulted in difficulty in maintaining the bifilament under the cot roll.

The draw ratio between the cot roll and the draw roll was 3.98 and the drawing speed was 3,050 feet/min. The yarn contained about 0.2 turns/inch twist and the drawn denier was 20. The weight of the yarn on the pirns was approximately 2 pounds. The yarn was then placed on a Leesona 553 Superloft false-twisting machine and false-twisted to a twist level of 31 turns/inch, at a heater temperature of 182°C and a spindle speed of 198,000 rpm. The yarn was fed into the twisting zone at a speed 6 percent slower than it was discharged from the twisting zone. The final package weighed 1 pound.

Round cross section polycaproamide yarn was prepared in a conventional manner, false-twisted with the same number of turns per inch as that for the bifilament yarns for use as a control yarn. These yarns were knit-

ted with a Textile Machine Works Mark IV 400-needle, 4 feed ladies' circular knit hosiery machine, into hosiery 35 inches in length which contained 2,100 courses throughout the full length of the hosiery, for an average of 60 courses per inch. The boarded hosiery contained at the ankle 74 wales per inch and 48 courses per inch. At the welt the hosiery contained 60 wales per inch and 66 courses per inch after boarding.

The polycaproamide yarns were boarded at a temperature of 118°C for bifilament yarns and 108°C for round cross section yarns, both temperatures being the maximum suitable for the particular cross section described in order to obtain the best stretch properties.

The bifilament yarns of this invention were knitted utilizing a tuck stitch on a Fidelity 2-feed circular knit machine for production of ladies' mesh knit hosiery for a comparison with hosiery of the same construction utilizing filaments having a triangular cross section.

After preboarding, the luster properties of these hosiery were determined as well as some special bifilament yarns prepared under conditions to produce different cross-sectional modifications which are described in example 17. The method for obtaining luster values listed in Table 1 is given in the description herein. The interpretations as to quality of the appearance are based on the dyed hosiery placed over a standard leg form and the values are recorded as the average of observations from a panel jury of 5 experienced colourists. Observations were made under fluorescent light and in bright daylight. Bright daylight assisted in showing the demarcation between sparkle and the "glace look" of the hosiery. It was noticed by the panel jury of judges, that daylight emphasized sparkle, but subdued internal lighting emphasized the "glace look." The ratings of the panel are listed in Table 1.

The true visual rating for the increase in sheen for the false-twist bifilament yarns as compared with the non-textured bifilament yarns was 200 to 300 percent greater at equal extension of a standard hosiery leg form. The panel jury of experienced colourists rated the bifilament yarns of this invention as having a sheer appearance value equal to between 10 to 12 denier for the 20 filament bifilament. This property is of significant value since it means that the bifilament yarns have an improvement in sheerness values of 165 percent without a loss in wearing properties as would normally be expected with a corresponding reduction in the denier typically required in round cross section hosiery to achieve the present sheerness values.

15 The improvement in sheerness is due to alignment of the concave surfaces facing each other at stitch crossing points so as to present the narrow edge to view.

All luster values listed in Table 1 were ascertained using a color eye fabric sample holder with a black 20 background and employing a Model D-1 "Color-Eye."

The boarded stockings were dyed in a conventional manner, dried by the tray method and placed in an Instron tester to evaluate the stretch properties of the hosiery. The hosiery were pretensioned at 1 percent of the 25 total Instron loading which was 500 grams minimum and 2,000 grams maximum. Thus, the pretensioning was between 5 and 20 grams, depending upon the degree of stretch in the hosiery being tested and the loads required to elongate the hosiery to 25 percent.

30 The Instron was equipped with G61-3C air-operated clamps gripping for a distance of 2 inches and the two jaws were separated from each other by a distance of 2 inches in lengthwise tests and 1 inch in the transverse tests. The rate of elongation was at 10 inches per minute on the loading part of the cycle and at the same rate on the unloading part of the cycle.

TABLE 1.—OPTICAL OR LUSTER PROPERTIES AS MEASURED ON THE BOARDED HOSIERY

| Example number | * <sup>3</sup> | Type cross section | Modifi-<br>cation ratio | Angle of bifilament intercept | Percent * <sup>1</sup><br>luster K/S by "color eye"     |                                                                            | Panel jury * <sup>2</sup> rating of the degree of silky sheen "glace look" |
|----------------|----------------|--------------------|-------------------------|-------------------------------|---------------------------------------------------------|----------------------------------------------------------------------------|----------------------------------------------------------------------------|
|                |                |                    |                         |                               | luster K/S by "color eye"                               | Panel jury * <sup>2</sup> rating of the degree of silky sheen "glace look" |                                                                            |
| 1.             | Br             | Bifilament         | 1.4                     | 62°                           | 6.0                                                     | No sheen, similar to round.                                                |                                                                            |
| 2.             | Br             | do                 | 1.65                    | 55°                           | 10.0                                                    | Good (A) subdued sheen.                                                    |                                                                            |
| 2A             | SD             | do                 | 1.70                    | 52.5°                         | 10-20%                                                  | greater cover over Example 6A.                                             |                                                                            |
| 3.             | Br             | do                 | 1.8                     | 49.2°                         | 12.0                                                    | Excellent strong "glace look" high sheen.                                  |                                                                            |
| 3A             | SD             | do                 | 1.95                    | 44°                           | 10-20%                                                  | greater cover compared with Example 6A.                                    |                                                                            |
| 4.             | Br             | do                 | 2.0                     | 42.6°                         | 14.0                                                    | Good (B) "glace look" with slight sparkle.                                 |                                                                            |
| 5.             | Br             | do                 | 2.5                     | 27°                           | 24.0                                                    | No "glace look," definite sparkle.                                         |                                                                            |
| 6.             | Br             | Round              | 1.0                     |                               | 4.5                                                     | No "glace look."                                                           |                                                                            |
| 6A             | SD             | do                 | 1.0                     |                               | 45.0                                                    | Dull without warmth.                                                       |                                                                            |
| 7.             | Br             | Triangular         |                         |                               | Heavy sparkle, too garish for most end-uses in hosiery. |                                                                            |                                                                            |
| 7A             | Br             | F-T triangular     |                         |                               | Heavy "sparkle."                                        |                                                                            |                                                                            |
| 8.             | Br             | F-T bifilament     | 1.7                     | 52.5°                         | 15.5                                                    | Good (A) subdued "glace look."                                             |                                                                            |
| 8A             | SD             | do                 | 1.8                     | 49.2°                         | Subdued sheen.                                          |                                                                            |                                                                            |
| 9.             | Br             | do                 | 1.9                     | 46°                           | 18.0                                                    | Excellent strong "glace look."                                             |                                                                            |
| 10.            | Br             | do                 | 2.05                    | 41°                           | 12.0                                                    | Subdued warm sheen.                                                        |                                                                            |
| 11.            | Br             | F-T round          | 1.0                     |                               | 3.5                                                     | No "glace look."                                                           |                                                                            |
| 12.            | Br             | F-T bifilament     | 2.5                     | 42°                           | 23.0                                                    | No "glace look," definite sparkle.                                         |                                                                            |

\*F-T=false twist.

\*<sup>1</sup> Luster is measured on the white boarded hosiery before dyeing.

\*<sup>2</sup> The panel jury of 5 experienced colourists' rating is based on observation of the dyed hosiery, and is as follows:

Excellent=Opalescent smooth silky high sheen, the preferred "glace look."

Good (A)=Opalescent silky sheen "glace look" present but slightly subdued.

Good (B)=An opalescent high sheen with the preferred "glace look" but some sparkle present.

\*<sup>3</sup> Br=bright hosiery.

\*<sup>4</sup> (Delestrant) SD=Semidull=0.3% by weight anatase TiO<sub>2</sub>.

TABLE 2.—FORCE IN GRAMS FOR HOSIERY EXTENDED LENGTHWISE AT THE INDICATED ELONGATIONS (+)

| Example number | Percent work of recovery                                   | Ankle elongation, percent |       |       |       |       |       | Percent work of recovery | Knee elongation, percent |     |     |     |       |       |       |
|----------------|------------------------------------------------------------|---------------------------|-------|-------|-------|-------|-------|--------------------------|--------------------------|-----|-----|-----|-------|-------|-------|
|                |                                                            | 3                         | 5     | 10    | 15    | 20    | 25    |                          | 3                        | 5   | 10  | 15  | 20    | 25    |       |
| 9.....         | Bifil false-twist Standard knit* stretch hosiery.          | 1 59.3                    | 18    | 27    | 48    | 78    | 113   | 145                      | 58.3                     | 18  | 22  | 32  | 45    | 58    | 75    |
|                |                                                            | 6 64.2                    | 10    | 16    | 34    | 63    | 100   | 136                      | 63.2                     | 8   | 12  | 23  | 36    | 52    | 70    |
| 11.....        | Round filament false-twist standard knit* stretch hosiery. | 1 43.7                    | 14    | 20    | 40    | 63    | 87    | 113                      | 54.0                     | 12  | 17  | 30  | 47    | 65    | 78    |
|                |                                                            | 6 50.5                    | 2     | 5     | 22    | 43    | 72    | 103                      | 56.4                     | 3   | 7   | 19  | 36    | 55    | 73    |
| 13.....        | Bicomponent standard knit* stretch hosiery.                | 1 44.6                    | 18    | 25    | 50    | 86    | 137   | 200                      | 53.2                     | 18  | 25  | 45  | 72    | 105   | 142   |
|                |                                                            | 6 48.2                    | 4     | 12    | 32    | 67    | 121   | 195                      | 58.1                     | 7   | 12  | 30  | 66    | 95    | 135   |
| 7A.....        | Triangular* cross section false-twist.                     | 6 52.0                    | 1     | 5     | 25    | 50    | 80    | 105                      | 47.1                     | 1   | 3   | 12  | 22    | 40    | 50    |
| 3.....         | Bifilament cross section standard knit* hosiery Nylon 6.   | 1 44.4                    | 300   | 400   | 800   | 1,200 | 1,700 | 2,300                    | 45.0                     | 300 | 500 | 850 | 1,320 | 2,000 | 1,800 |
|                |                                                            | 6 59.0                    | 50    | 60    | 300   | 700   | 1,300 | 2,100                    | 60.4                     | 50  | 350 | 800 | 1,500 | 1,600 |       |
| 6.....         | Round cross section Standard knit* hosiery Nylon 6.        | 1 39.0                    | 400   | 650   | 1,300 | 2,000 | 2,800 | 3,600                    | 41.0                     | 300 | 500 | 950 | 1,350 | 1,800 | 2,300 |
| 14.....        | Bifilament cross section Mesh-knit++ —Nylon 6.             | 1 40.6                    | 450   | 800   | 2,000 | 3,400 | 5,000 | 6,500                    | 45.7                     | 200 | 350 | 650 | 1,100 | 1,700 | —     |
|                |                                                            | 6 57.5                    | (***) | (***) | 500   | 1,800 | 3,700 | 6,200                    | 61.2                     | —   | 300 | 600 | 1,300 | —     |       |
| 7.....         | Triangular cross section Mesh-knit++—Nylon 6, 6.           | 1 38.7                    | 500   | 1,000 | 2,200 | 3,520 | 4,900 | 6,250                    | 41.1                     | 200 | 320 | 700 | 1,200 | 1,800 | —     |
|                |                                                            | 6 58.5                    | (**)  | (**)  | 400   | 1,700 | 3,600 | 5,800                    | 58.8                     | —   | 200 | 600 | 1,350 | —     |       |

\*Standard knit, plain or jersey stitch.

\*\*Too small to read on Instron on 10,000 gram load scale.

\*\*\*Load too small to show on chart.

+The values in the table are all expressed in grams with the exception of work of recovery.

++Mesh knit=tuck stitch.

Work of recovery is the ratio of recoverable work to the total work required to strain a fiber or fabric a specified amount under a given program of strain rate. In this case, it was determined at 25 percent elongation 15 seconds forward cycle, 15 seconds return and was calculated according to ASTM D-1774-64, ASTM Standards (1964) part 25, pp. 428-432.

All values for Tables 2, 3, 4 and 5 were measured using Instron G61-3C 2-inch rubber faced air operated jaws clamped with 60 pound pressure. The cross head and gage length were the same and a 25 percent elongation was achieved in 15 seconds. There was 2 inches of hosiery between the clamped jaws and lengthwise tests and 1 inch of hosiery between clamped jaws in the transverse or width tests.

The bicomponent and triangular yarns evaluated herein are sold commercially.

The elastic properties of the hosiery on lengthwise extension are given in Table 2. As can be seen the ankle and the knee areas were selected since these are the areas of greatest wrinkle problems in ladies' hosiery.

Referring to the results shown in Table 2, it can be noted that the bifilament false-twist yarns have the highest work of recovery of all yarns tested and the improvement in terms of work of recovery is the greatest after 6 cycles when compared to other types of yarns tested as indicated by Example 9. Most significant in the stress-strain curve was the stress force at an elongation of 3 percent. It can be noted that the hosiery of Example 9 had a stress force of 16 grams which was 250 to 500 percent higher loading in the ankle area at 3 percent elongation than the round cross section false-twisted yarn (Example 11) or bicomponent stretch hosiery (Example 13). Without false twist, the bifilament cross section, plain knit or jersey knit hosiery (Example 3) may be compared with the round cross section yarn (Example 6). The work of recovery on the first cycle is 44.4 percent or 10 percent higher for the bifilament cross section than the round which would indicate definitely improved wrinkle resistance. In Table 2, it can be observed further that the bifilament cross section yarn (Example 3) has greater elasticity after 6 cycles of extension than the round cross section of plain knit and less force is required to extend it to 25 percent. Indeed, the stress forces are about one-half that required to extend round cross section yarn of an equal denier. After six cycles of extension the bifilament cross section plain knit hosiery has a stress force of 50 grams which indicates excellent capacity to retain its shape, whereas the

round cross section has an immeasurably small value. 20 Bifilament yarns containing 0.3 percent  $TiO_2$  and 2 percent  $TiO_2$  were converted to false-twist yarns similar to that described for Example 9 and exhibited similar elastic properties in test hosiery as that illustrated in Table 2 for Example 9. Likewise, bifilament cross section yarns containing 0.3 and 2.0 percent of  $TiO_2$  were converted to standard jersey knit hosiery. The bifilament yarns containing  $TiO_2$  exhibited similar elastic properties as that of Example 3. The bifilament false-twist yarn of Example 9 might be additionally compared with the triangular cross section false-twist Yarn of Example 7A in the form of similar hosiery. As can be observed, the work of recovery for the triangular cross section false-twist yarn is significantly less than bifil false-twist yarns and the elongation after six cycles 30 at 3 percent elongation was 1 gram compared with 10 grams, or about 10 percent of that obtained for the bifilament yarns at the ankle section of the hosiery.

Likewise, the triangular cross section yarn hosiery in the knee section had significantly less work of recovery 40 and very low load to 0 loads at 3 percent elongation than did the bifilament cross section of Example 9 which had a stress force of 9 grams when tested in the knee section. Thus, it should be expected that the triangular cross section yarns generally would have greater 45 problems with sagging and wrinkling than would the bifilament yarns of this invention.

Examples 14 and 7, respectively, show a comparison 50 of bifilament cross section with triangular cross section in a mesh knit stocking. Generally, the elastic properties are approximately equivalent to the triangular cross section in the mesh knit hosiery. It is believed that failure to show equivalent advantages here may be due to tuck knit stitch on long courses having reduced twist and, consequently, this type stitch interferes with the 55 ability of this yarn to twist at stitch doubling areas.

The data for Examples 9, 11, and 13 are shown 60 graphically in FIGS. 15, 16 and 14, respectively, and the picture of the knit hose of Example 9 is shown in FIG. 8, Example 11 in FIG. 10, and Example 13 in FIG. 12.

The bifil cross section mesh knit hosiery has 5 to 10 percent greater work of recovery in the knee section than does triangular cross section mesh knit yarn, both 65 being made employing a tuck knit stitch. After six cycles, the bifil cross section appears to retain 50 percent more force in the knee section at 10 percent elongations. However, in Table 3, it can be observed that in

the transverse direction, the bifilament mesh knit hosiery after six cycles, has a stress force of 10 grams at 3 percent elongation and at the knee section and at the welt section. Additionally, after six cycles, the power of recovery (see Table 4) of the bifil mesh knit in the lengthwise knee area was 150 grams or 150 percent greater than that for the triangular cross section.

In Table 3, bifilament false-twist yarns (Example 9) are superior to round false-twist yarns (Example 11) and bicomponent round cross section (Example 13) in plain knit in a transverse direction over the entire range of elongation and at 25 percent elongation, especially after 6 cycles of extension. The values vary between 200 percent and 100 percent higher for Example 9 than for Examples 11 and 13 in the transverse direction. For bifilament plain knit hosiery (Example 3) as compared with round plain knit standard hosiery (Example 6) it can be observed that the transverse force elongation values are much higher and would represent a more comfortable extension force than that obtained for round cross section. After six cycles, the values for the bifilament were adequate to avoid wrinkling and obtained a smooth fit in the ankle region and in the knee region.

Example 7A, triangular cross section false-twist yarns had similar properties in transverse direction to that of the bicomponent yarns up to a 10 percent elongation; however, at 10 percent elongation and above, very rapid loading ensued which indicated a lower degree of elasticity for the triangular cross sections of this yarn.

Table 4 illustrates a more significant part of the elastic properties. In this case the yarn was extended to 25 percent elongation and allowed to return to 12½ percent elongation and the force in grams ascertained at this point by reading from the chart. This value is designated as the "power of recovery," and is frequently referred to as the muscle power of the fabric and is probably a more significant value than is the forward extension part of the cycle. As can be observed in Table 4, 10 bifilament false-twist stretch hosiery (Example 9) after six cycles of lengthwise stretch has a power of recovery of 25 grams or 300 percent greater force at the ankle as compared with the bicomponent round cross section false-twist stretch yarn. Additionally, the bifilament 15 yarn has significantly higher values in the knee section.

In Example 9, bifilament false-twist stretch hosiery after six cycles of lengthwise stretch has at least 200 percent greater force at the ankle as compared with a triangular cross section (Example 7A) false-twist 20 stretch hosiery of identical construction.

A similar improvement for Example 9 over Example 11 and Example 13 can be observed for the "power of recovery" in the transverse direction. The power of recovery for bifilament yarn (Example 3) in the knee section 25 is 125 grams or approximately twice that of the round cross section (Example 6) in the lengthwise direction. The power of the recovery of 175 grams for bifilament cross section mesh knit yarn (Example 14) is approximately twice that for the triangular cross section 30 mesh knit hosiery (Example 7) after 6 cycles of extension.

TABLE 3.—HOSIERY PHYSICAL PROPERTIES—TRANSVERSE

| Example No.                                 | Number of cycles | Ankle elongation, percent |    |     |     | Below-welt-thigh area elongation, percent |    |    |     |
|---------------------------------------------|------------------|---------------------------|----|-----|-----|-------------------------------------------|----|----|-----|
|                                             |                  | 3                         | 5  | 10  | 25  | 3                                         | 5  | 10 | 25  |
| 9..... Bifil F.T.*.....                     | 6                | 5                         | 7  | 12  | 50  | 5                                         | 7  | 15 | 60  |
| 11..... Round F.T.*.....                    | 6                | 1                         | 3  | 5   | 26  | —                                         | 2  | 7  | 50  |
| 13..... Bicomponent*.....                   | 6                | —                         | 3  | 6   | 15  | 3                                         | 5  | 10 | 25  |
| 7A..... Triangular cross section F.T.*..... | 6                | 2                         | 5  | 125 | 3   | —                                         | —  | —  | —   |
| 3..... Bifil plain*.....                    | 6                | 5                         | 10 | 50  | 190 | —                                         | 5  | 70 | 550 |
| 6..... Round cross section*.....            | 6                | 4                         | 10 | 100 | 470 | —                                         | 5  | 80 | 460 |
| 14..... Bifil mesh knit**.....              | 6                | 5                         | 10 | 40  | 380 | 10                                        | 10 | 30 | 570 |
| 7..... Triangular mesh knit.....            | 6                | 5                         | 10 | 35  | 185 | 5                                         | 8  | 25 | 270 |

\* Plain or jersey knit.

\*\* Mesh knit or tuck stitch hosiery.

NOTE.—F.T.=False twist.

TABLE 4.—"POWER OF RECOVERY"—EXTENSION TO 25% ELONGATION WITH MEASUREMENT OF LOAD ON RETURN TO 12½% ELONGATION

| Example number                                      | Number of cycles | Lengthwise of hosiery |       |        | Transverse or width direction of hosiery |       |        |
|-----------------------------------------------------|------------------|-----------------------|-------|--------|------------------------------------------|-------|--------|
|                                                     |                  | Ankle*                | Knee* | Thigh* | Ankle*                                   | Knee* | Thigh* |
| 9..... Bifil false twist**.....                     | 1                | 27                    | 20    | 10     | —                                        | —     | —      |
|                                                     | 6                | 25                    | 15    | 7      | 10                                       | 8     | 7      |
| 11..... Round cross section false twist**.....      | 1                | 14                    | 12    | 7      | —                                        | —     | —      |
|                                                     | 6                | 8                     | 8     | 5      | 3.5                                      | 3     | 3      |
| 13..... Bicomponent round cross section**.....      | 1                | 12                    | 18    | (***)  | —                                        | —     | —      |
|                                                     | 6                | 7                     | 12    | (***)  | 3.5                                      | 5     | 5      |
| 7A..... Triangular cross section false-twist**..... | 6                | 12                    | 7     | —      | —                                        | —     | —      |
| 3..... Bifil hosiery**.....                         | 1                | 250                   | 150   | 130    | —                                        | —     | —      |
|                                                     | 6                | 150                   | 125   | 100    | 20                                       | 40    | 50     |
| 6..... Round hosiery**.....                         | 1                | 225                   | 100   | 60     | —                                        | —     | —      |
|                                                     | 6                | 150                   | 60    | 50     | 30                                       | 20    | 10     |
| 14..... Bifil mesh knit.....                        | 1                | 350                   | 200   | 350    | —                                        | —     | —      |
|                                                     | 6                | 250                   | 175   | 250    | 35                                       | 26    | 26     |
| 7..... Triangular mesh knit sparkle yarn.....       | 1                | 300                   | 150   | 150    | —                                        | —     | —      |
|                                                     | 6                | 200                   | 100   | 125    | 25                                       | 20    | 12     |

\*Force in grams after extension to 25% elongation and return to 12½% elongation is designated the "power of recovery."

\*\*Plain or jersey knit.

\*\*\*No data.

Table 5 illustrates the maximum elongation of stretch hosiery at fixed stress loads. As can be observed in Table 5, Example 9 bifilament false-twist stretch hosiery were superior to round cross section false-twist stretch hosiery (Example 11) and Example 13 bicomponent round cross section stretch hosiery. It can be noted on a single cycle that both false-twist yarns were substantially superior to bicomponent round stretch hosiery in their total elongation. Thus, it can be concluded that the major differences between the two cross sections are best illustrated after repetitive cycling.

TABLE 5.—MAXIMUM ELONGATION OF HOSIERY STRETCH AT ANKLE

| Example number |                                     | Percent elongation—after one cycle |                 |                                        |                 |
|----------------|-------------------------------------|------------------------------------|-----------------|----------------------------------------|-----------------|
|                |                                     | 500-gram load                      | 1,000-gram load | Where yield point occurs <sup>5*</sup> | 2,000-gram load |
| 9              | Bifill false-twist stretch hosiery. | 85                                 | 101             | 84                                     | 120             |
| 11             | Round false-twist stretch hosiery.  | 84                                 | 98              | 80                                     | 118             |
| 13             | Bicomponent round stretch hosiery.  | 36                                 | 56              | 36                                     | 80              |

\*This value was obtained in the test procedure similar to that for the yield point in yarns where a straight line is taken along initial load line, then a similar straight line is drawn at maximum loading or stress to bisect the first line drawn and then a straight line from this intercept with the stress-strain line drawn by the Instron. This intercept point is called the "yield point."

From Tables 2 through 5 the following general conclusions may be drawn:

1. Bifilament false-twist yarns (Example 9) on repetitive cycling have substantially improved elastic properties as compared with Examples 11, 7A and 13 over the entire range of tests evaluated.

2. Bifilament cross section yarn in standard knit hosiery (Example 3), as compared with round cross section in standard knit hosiery, has some slightly improved properties after one cycle and significantly improved properties after six cycles over the entire range evaluated.

3. Bifilament cross section mesh knit hosiery (Example 14) has equal properties over most tests employed and slightly to significantly improved properties after six cycles of testing as compared with a triangular cross section mesh knit hosiery.

It is observed that the bifilament yarns (Examples 2, 3, 8, 9 and 10) in a 20-denier exhibited approximately the same sheerness of that observed for a 10-denier monofilament. This is because bifilament yarns where they cross at the stitch point present the narrow edge of the bifilament to view. Thus, at the point of maximum abrasion or compression one presents the best geometric area for breaking resistance while the minimum geometric area is presented to the eye, thereby achieving sheerness and simultaneously good wearing qualities of the hosiery.

Panel jury tests of 20 women in wear tests of a single size hosiery made of false-twist bifilament yarns (Example 9) rated them as sag-free having excellent wearing qualities and having exceptional aesthetic qualities in appearance. They rated the comfort fit over an entire range of leg sizes of 8-1/2 to 10-1/2 as excellent. The wearing qualities were quite superior to other hosiery such as Example 11, false-twist round cross section hosiery, Example 7A triangular cross section false-twist hosiery, and Example 13 bicomponent standard knit

stretch hosiery. The bicomponent hosiery in all examples were composed of nylon 6,6 as the sheath portion which is about 35 percent by weight and nylon 6,10-6,6 copolymer in the core portion generally in the kidney shape as 65 percent of the total.

The above hosiery fashioned from bicomponent and triangular cross-section yarns were purchased for comparative evaluations.

#### EXAMPLE 15

Bicomponent yarn was prepared by the procedures described in Examples 1-14 except nylon 6,6 was employed. The bifilament yarn was false-twisted and compared with similar hosiery made from false-twist round cross section yarn. These were tested for work of recovery, and stress-strain curves similar to those indicated in Tables 2, 3, 4, and 5. The bifilament hosiery made from polyhexamethylene adipamide showed approximately equivalent improvement in all physical properties and in luster effects as that already described for polycaproamide when compared with the round cross section made under identical conditions except with respect to the spinnerettes employed. The spinning temperature was maintained at about 280°C to produce a glace look from the polyhexamethylene adipamide (nylon 6,6).

#### EXAMPLE 16

Poly[bis(para-aminocyclohexyl)methane dodecamedes] was spun at a temperature of 290°C through bifilament spinnerettes of the type illustrated in FIG. 1 and was drawn at a draw ratio of 3. The drawn yarn had a density of 1.001; a moisture absorption of 3 percent at 65 percent relative humidity and a glass transition temperature of greater than 100°C. This yarn was also prepared in round cross section. The same improvement in elastic properties for bifilament cross section in hosiery after twisting over the control in round cross section was noted; however, the elastic properties as compared with polycaproamide and polyhexamethylene adipamide was approximately twice as great in the force in grams at low elongations of 3 and 5 percent. The work of recovery was between 10 and 15 percent higher than that indicated for polycaproamide. The muscle value or power of recovery was approximately 100 percent greater than the polycaproamide listed as Example 9, Table 4, for the ankle, knee and thigh dimensions.

These values are desirable for support hosiery but too high for conventional stretch hosiery, for a comfortable fit.

#### EXAMPLE 17

A series of runs were made employing polyamides of relative formic acid viscosity of 25 to 90 using a spinnerette of the type illustrated in FIG. 1. A range of temperatures from 250° to 290°C were evaluated. The distance between the spinnerette orifices tested was from 0.9 to 4.0 mils. Heated quench air immediately below the spinnerette was evaluated in the range of 260° to 350°C and the velocity of the quench air in the vicinity of one-fourth to one-half inch from the spinnerette face was evaluated in the range of 0 to 8 standard cubic feet/minute/25 pounds per hour throughput. Polymer throughput was evaluated at a high rate, 8 grams/minute/bifilament and at a low rate of 2 grams/minute/bifilament. The spinnerette orifice length of 20 to 150 mils was evaluated.

In Table 6 are the results of these evaluations in order to optimize the "glace look."

entation of reflection which in turn increases the "glace look."

TABLE 6.—PROCESS FOR CONTROL OF MODIFICATION RATIO

| Significance level                                      | Approx. rel. effect on mod. ratio, percent as compared with No. 1 | Assuming value on left increases effect on mod. ratio | "Glace look"     |                  | "Scintilla look" |              |
|---------------------------------------------------------|-------------------------------------------------------------------|-------------------------------------------------------|------------------|------------------|------------------|--------------|
|                                                         |                                                                   |                                                       | Range            | Preferred        | Range            | Preferred    |
| Polyamide relative formic acid viscosity                | 1                                                                 | 100 Increases                                         | 25-65            | 40-60            | 40-90            | 58-75        |
| Mils between spinnerette orifices                       | 2                                                                 | 90 do                                                 | 0.9-3.0          | 1.5-2.5          | 2.5-4.0          | 2.5-3.5      |
| Temperature, °C.                                        | 3                                                                 | 60 Decreases                                          | 260-280          | 265-275          | 255-290          | 260-280      |
| Heated quench, °C. medium immediately below spinnerette | 4                                                                 | 30-40 do                                              | 260-350          | 300-350          |                  |              |
| Quench air rates in the vicinity of the spinnerette     | 5                                                                 | 25 Increases                                          | 0.1-1.0 s.c.f.m. | 0.1-0.5 s.c.f.m. | 4-8 s.c.f.m.     | 6-8 s.c.f.m. |
| Polymer throughput                                      | 6                                                                 | 20 Decreases                                          | High*            | 4.58 g.p.m.      | Low**            | Low          |
| Spinnerette orifice capillary:                          |                                                                   |                                                       |                  |                  |                  |              |
| Length effects                                          | 7                                                                 | 10-15 Increases                                       | Short            | Short            | Long             | Long         |
| Length in mils                                          |                                                                   |                                                       | 8-80             | 8-150            | 8-150            | 20-150       |
| Length/diameter                                         | (***)                                                             |                                                       | 0.8-3.0          | 0.8-2.0          | 2-20             | 2-10         |

\*4-8 grams per minute per bifil filament.

\*\*2-6 grams per minute per bifil filament orifice.

\*\*\*Capillary length is proportional to diameter; thus a larger diameter requires a longer length. A better characterization of this is the spinnerette capillary length divided by the spinnerette capillary diameter.

Since tricot knits have a stitch very similar to the plain knit, e.g., jersey knit stitch, fabric made by tricot knitting exhibits similar elasticity utilizing the bifilament yarn of this invention. Generally, it can be said that tricot fabrics have about 50 to 60 percent less elasticity than jersey knit products. By utilizing bifilament false-twisted yarns one can achieve approximately equivalent elasticity in the tricot knit wear as that obtained for jersey knits of round cross section which greatly enhances the elasticity of tricot knits. These bifilament yarns find utility in womens' slacks, in swim wear, where the characteristics of high sheen, high gloss combined with the elastic properties considerably enhances the utility of the textile article made from bifilament yarns.

Additionally, particularly where sheer fabrics and styling are desirable, such as in intimate wear, e.g., nightgowns, housecoats, lounge suits, negligees, peignoirs, and the like, these bifilament textile articles have high utility. Tricot knit fabrics and other flat fabrics may be further modified in appearance by employing processes known as wet-calendering and frictioning calendering. Generally pastel color favors the "glace look". The so-called ice or basic dyes insure that the "glace-look" is maintained in the finished dyed article. In mixed fabrics, dark dyes decrease the glace look and bright dyes increase the glace look. Polyamides having an amine end group of 25 or less may be dyed at a pH of 7 with basic dyes and an amine group of 40 to 50 using a pH of 8 with basic dyes. Using an amine end group as high as 70 to 75 millequivalents per kilogram of polymer, polyamides may be dyed at a pH of 8.5 with basic colors. Other means of increasing the glace look are plaiting of glace look yarn on the front of a dark-colored backing yarn. If the low modification ratio bifilament yarns of this invention are employed in jersey knit articles and only in the wales essentially the same glace look is obtained as if the bifilament yarn were included throughout the textile article. However, this is at a considerable loss in the elastic properties of the textile article. A considerable increase in the "glace look" can be obtained by doubling the number of yarn ends in the wales. An opposite effect is obtained if one doubles the number of yarn ends in the courses, since this tends to emphasize sparkles.

By alternating wales using bifil yarns, the pattern responds to vertical light which tends to highlight the ori-

25 It has been found that the high luster and high sheen characteristics of the bifilament yarns of this invention, whether false-twisted or other texturing systems are employed, the reflectivity is relatively unchanged after washing from the original textile article prior to soiling. Therefore, the apparent soiling of such fabrics is largely overcome by a minor reduction in the sheen and the general appearance with respect to soiling is considerably 30 superior to other cross sections such as round, triangular and the like although treated in the similar manner. This property is of particular value in white intimate wear and in pastel colors which would otherwise show considerable soiling in cross sections employed 35 heretofore in the prior art.

While the production of the bifilament yarn product of the present invention has been illustrated utilizing separate orifices, those skilled in the art will recognize that other types of orifices may be employed. For example, two holes connected by a thin slot may be used through proper control of spinning conditions which achieve a bifilament as described herein.

We claim:

1. A polyamide bifilament yarn comprised of two lobes interconnected by symmetrically opposed concave sides which form an oblong yarn cross section characterized by an intercept angle  $\theta$  ranging from 41 to 54 degrees.
2. The yarn of claim 1 further characterized by a modification ratio of between 1.65 and 2.05.
3. The yarn of claim 1 in which the lobes have substantially circular portions of equal diameter connected by the concave sides, said circularity being greater than 0.9.
4. The yarn of claim 3 in which the polyamide is selected from the group consisting of polycaproamide, polyhexamethylene adipamide and poly[bis(p-aminocyclohexyl)methane dodecamide].
5. The yarn of claim 3 in which the denier is from 1 to 100.
6. A jersey-knit fabric prepared from the yarn of claim 3 in which the fabric has a luster value between 8 and 15 (K/S  $\times$  100) units.
7. The jersey-knit fabric of claim 6 in which the yarn has at least 30 turns per inch false twist and the fabric has a luster value between 14 and 21 (K/S  $\times$  100) units.

\* \* \* \* \*